# EUROPEAN PATENT APPLICATION

(11) **EP 4 786 648 A1**
(43) Date of publication of application: **05.08.2026**
(21) Application number: 26155320.0
(22) Date of filing: 30.01.2026
(51) Int. Cl.: C23C 28/00, C23C 4/02, C23C 4/073, C23C 4/134, C23C 4/18

(54) **PROTECTIVE COATING FOR COMPONENTS EXPOSED TO HIGH TEMPERATURES**

(30) Priority: 31.01.2025 IT 202500001815
(71) Applicant: ANSALDO ENERGIA S.p.A., 16152 Genova (IT)
(72) Inventor: GUALCO, Giuseppe Carlo, 16152 GENOVA (IT); VACCHIERI, Erica, 16152 GENOVA (IT)
(74) Representative: Studio Torta S.p.A.

(57) **Abstract**

A thermal barrier fixed to a surface of a material exposed to high temperatures comprising a bond coat layer fixed to the surface of the material to be protected and a thermal insulating ceramic layer fixed to the bond coat layer. The bond coat comprises a first and a second layer distinct from each other and both composed of a MCrAlY+N alloy; wherein M is selected from Ni and Co, and N is selected from the group composed of Re, Ir, Si, Ta and Pt; the first and second layers have a different % by weight of the elements.

## Description

### CROSS-REFERENCE TO RELATED APPLICATIONS

This patent application claims priority from Italian patent application no. 102025000001815 filed on January 31, 2025, the entire disclosure of which is incorporated herein by reference.

### TECHNICAL FIELD

The present invention relates to a protective coating for components exposed to high temperatures, such as components of a gas-turbine engine.

### BACKGROUND ART

As is known, the operating environment inside a gas-turbine engine is both thermally and chemically hostile to the materials that are exposed to it.

A long-established solution has been to protect the materials with a thermal barrier coating (TBC) system. The latter generally includes a thermal insulating ceramic layer applied to the substrate by means of a bonding layer. Hereinafter, in the present document, the bonding layer will be referred to by the term "bond coat", which is commonly adopted in the industry.

Metal oxides, such as for example zirconium oxide (ZrO2), which is partially or completely stabilized by yttrium oxide (Y2O3), were employed for the thermal insulating ceramic layer. In recent years, more complex oxides, such as for example lanthanum, cerium, neodymium, or ytterbium and gadolinium zirconates, have also been used instead of yttrium oxide, although in limited applications. The ceramic layer can be deposited by means of different deposition techniques, such as air plasma spray (APS), physical vapor deposition (PVD), electron beam physical vapor deposition (EBPVD), suspension plasma spray (SPS). APS is often preferred over other deposition techniques due to the low cost of equipment and the ease of application and masking. In particular, the adhesion mechanism for plasma-sprayed ceramic layers takes place via mechanical interlocking with a bond coat having a relatively rough surface, in particular with a Ra between about 9 and about 19 µm.

Bond coats are typically formed from an oxidation-resistant alloy such as MCrAlY+N, or from a diffusion aluminide or platinum aluminide forming an oxidation-resistant intermetallic, or a combination of both.

In the MCrAlY+N alloy, M is iron, cobalt, and/or nickel, while N denotes one or more possible, but not necessary, elements selected from the group composed of silicon, rhenium, tantalum, iridium, and/or others, with specific functions, such as for example the reduction of the aluminum diffusion coefficient within the coating.

Bond coats made with such compositions protect the substrate by forming an oxidation barrier for the substrate itself. In particular, the aluminum content of these bond coats allow the slow growth of a dense layer of adhesive aluminum oxide (alumina scale) at high temperatures. This oxide scale protects the bond coat from further oxidation and improves the bond between the ceramic layer and the bond coat itself.

The oxidation of the bond coat cannot be avoided because the thermal insulating ceramic layer is unable to avoid the diffusion of oxygen in the solid state or its permeation through porosity and microcracks, which must be present to reduce the thermal conductivity and brittleness of the ceramic coating.

The chemical composition of the bond coat results from a compromise between different needs, in terms of relative quantities of the several elements. In fact, a bond coat must have many properties that are not perfectly compatible with each other. These properties refer to (a) the chemical compatibility with the base material; (b) the thermal expansion coefficient similar to that of the base material; (c) the lowest possible transition temperature from ductile to brittle; (d) the high resistance to crack formation, low crack propagation velocity, and high resistance to thermal fatigue; (e) the high resistance to hot corrosion (this property is not crucial in many modern very high-efficiency turbines); (f) the high resistance to oxidation (which becomes even more important if the overlying thermal insulating ceramic layer detaches, because the anchor temperature rises to much higher values, even 200 °C higher); (g) the formation of a dense and highly adhesive oxide scale, adapted to tightly maintain the adhesion of the overlying thermal insulating ceramic layer; (h) the resistance to damage and contamination due to post-coat deposition machining processes (general thermal treatments and, in particular, brazing and cooling hole machining).

While properties (a)-(d) require a limited aluminum content (about <5% by weight) and ensure excellent compatibility with the base material, properties (f)-(h) require a high aluminum content (>8% by weight) and are aimed at achieving an excellent bond coat surface behavior. Finally, property (e) requires a high chromium content (>28% by weight), which is not, however, compatible with properties (f)-(h).

For example, a bond coat with an aluminum quantity >12% showed excellent resistance to oxidation and excellent adhesion of the thermal insulating ceramic layer but, at the same time, showed poor fatigue resistance, with the formation of cracks which propagated to the base material. In contrast, a bond coat with an aluminum content <4% showed strong reactivity with the carbon present in the atmosphere of a thermal treatment furnace, with the formation of a reaction layer on its surface, which was poorly adapted for the adhesion of the thermal insulating ceramic layer.

One of the problems that research had to address in this field related to the premature detachment of significant parts of the thermal insulating ceramic layer after a number of operation hours lower than expected. This detachment necessarily involves an overheating of the areas that are no longer protected, in some cases leading to the formation and propagation of cracks in the base material.

Generally, since hot corrosion was a phenomenon as feared as oxidation, bond coats have always had a composition which was relatively poor in aluminum (<7%) and very rich in chromium (about 30% or slightly lower) . Furthermore, in order to ensure good performance in terms of anchoring of the thermal insulating ceramic layer to the bond coat, a thin (between 0.05 and 0.1 mm) but rougher layer of the same composition was deposited onto the bond coat.

For a more complete understanding of the problem that the present invention aims to solve, the evolution in the bond coat deposition technique must be taken into consideration. For productivity reasons, very often the vacuum plasma spray technique, used for both the main layer in contact with the material to be protected and the rough surface layer, has been replaced by the HVOF (High Velocity Oxygen Fuel) technique for the main dense part and by the air plasma spray technique for the rough surface layer (which is called APS flash; flash because it is thin). Such replacement is still ongoing, and the number of parts coated with vacuum plasma spray is still decreasing.

Despite representing a benefit from a production viewpoint, the use of HVOF and air plasma spray techniques has nevertheless resulted in problems relating to premature detachment of the thermal insulating ceramic layer. In fact, the rough surface layer, when deposited with HVOF employing a coarse powder, does not often achieve optimal roughness, while when deposited with the APS flash technique, it tends to form mixed oxides, which have poor adhesion when its composition is low in aluminum. Furthermore, instead of a dense aluminum oxide scale, such poorly adhesive mixed oxides also form, and often especially, at relatively low temperatures, even as low as 750 °C.

There was a need for a technical solution that could ensure the adhesion of the thermal barrier to the base material for periods longer than those of the prior art, regardless of the techniques with which the bond coat thereof is deposited.

### DESCRIPTION OF THE INVENTION

In order to meet the above-mentioned need, the inventors of the present invention made a bond coat composed of two distinct layers consisting of two different chemical compositions. In this way, the functions of the bond coat have been separated into the two layers composing it.

An object of the present invention is a thermal barrier fixed to a surface of a material exposed to high temperatures; said thermal barrier comprising a bond coat layer fixed to the surface of the material to be protected and a thermal insulating ceramic layer fixed to the bond coat layer; said thermal barrier being characterized in that said bond coat comprises a first and a second layer distinct from each other and both composed of a MCrAlY + N alloy; wherein M is selected from Ni and Co, and N is selected from the group composed of Re, Ir, Si, Ta and Pt; said first and second layers having a different % by weight of the elements;
- said first layer being in contact with said surface of the material to be protected and composed of 2 to 7% by weight of Al, 0.5 to 2% by weight of Y, 10 to 35% by weight of Cr, 0 to 5% by weight of N and a % by weight of M to complete 100;
- said second layer being fixed to said first layer and composed of 8 to 14% by weight of Al, 0.5 to 2% by weight of Y, 10 to 20% by weight of Cr, 0 to 5% by weight of N and a % by weight of M to complete 100;
- said first layer having a thickness between 100 and 500 µm, preferably between 180 and 300 µm, and said second layer having a thickness less than or equal to 150 µm, preferably between 10 and 70 µm.

Preferably, said second layer has a surface with a roughness Ra between 8 and 23 µm, more preferably between 12 and 20 µm.

Preferably, said first layer is composed of 4 to 6% by weight of Al, 0.5 to 1% by weight of Y, 20 to 28% by weight of Cr, 0 to 2.5% by weight of N and a % by weight of M to complete 100.

Preferably, said second layer is composed of 10 to 12% by weight of Al, 0.5 to 1% by weight of Y, 13 to 17% by weight of Cr, 0 to 2.5% by weight of N and a % by weight of M to complete 100.

### BRIEF DESCRIPTION OF THE DRAWINGS

Hereafter embodiments of the present invention will be described for illustrative and non-limiting purposes together with the accompanying figures, in which:
- Figure 1 is a schematic view of the thermal barrier according to the invention; and
- Figure 2 is a chart where the experimental results of the cyclic oxidation tests are reported.

### PREFERRED EMBODIMENT OF THE INVENTION

In the figure, reference numeral 1 denotes, as a whole, a thermal barrier fixed by deposition to the surface 2 of a material 3 to be protected against high temperatures.

The thermal barrier 1 comprises a thermal insulating ceramic layer 4 and a bond coat layer 5, which is composed of a first layer 6 fixed to the surface 2 of the material 3 to be protected, and a second layer 7 fixed to a surface 8 of the first layer 6 on the opposite side to the material to be protected.

The first layer 6 and the second layer 7 are made with a MCrAlY + N alloy; wherein M is selected from Ni and Co, and N is selected from the group composed of Re, Ir, Si, Ta and Pt.

The first 6 and second 7 layers can be discerned from each other by the different % by weight of the elements in the alloy.

The first layer 6 has a composition made up of 2 to 7% by weight of Al, 0.5 to 2% by weight of Y, 10 to 35% by weight of Cr, 0 to 5% by weight of N and a % by weight of M to complete 100.

Materials corresponding to the above-described composition relating to the first layer 6 are commercially available under the trade names Amperit 418, NI535, Amdry 2231, CO 301, Amperit 422, Amdry 995, Amperit 415, and CO 210.

The second layer 7 has a composition made up of 8 to 14% by weight of Al, 0.5 to 2% by weight of Y, 10 to 20% by weight of Cr, 0 to 5% by weight of N and a % by weight of M to complete 100.

Materials corresponding to the above-described composition relating to the second layer 7 are commercially available under the trade names NI 832, Amperit 436, Amdry 2464, Amperit 429, NI 944, Amperit 428, NI 937, and Amperit 416.

The inventors made a series of specimens reproducing the thermal barrier according to the invention and tested their effectiveness compared to specimens reproducing the thermal barriers according to the prior art.

For a more complete evaluation of the advantages of the invention, the bond coat of the specimens was produced with different deposition techniques.

The deposition techniques used in the examples were low pressure plasma spray (LPPS) for both layers, or high velocity oxygen fuel (HVOF) for the first layer and air plasma spray (APS) for the second layer.

Table I below reports the compositions of the bond coats of the specimens made together with an indication of the technique used.

**Table I**

| Specimen | First layer | Second layer |
|---|---|---|
| Bond coat according to the invention | | |
| 1 | Amperit 418.117 (LPPS) | Amperit 436 (LPPS) |
| 2 | Amperit 418.117 | Amperit 429 (LPPS) |
| | (LPPS) | |
| 3 | Amperit 418.724 (HVOF) | Amperit 436 (APS) |
| 4 | Amperit 418.724 (HVOF) | Amperit 429 (APS) |
| 5 | Amperit 422 (HVOF) | Amperit 429 (APS) |

| Comparison bond coat | | |
|---|---|---|
| 6 | Amperit 418.11720 (LPPS) | Amperit 418.715 (LPPS) |

The thickness of the first layer was equal to 180 µm and the thickness of the second layer was equal to 75 µm.

The base material used for the specimens 1-6, and on which the respective bond coats were deposited, was the nickel-based superalloy MarM247.

Furthermore, the same thermal insulating ceramic layer consisting of zirconia partially stabilized with 7% by weight of yttria was deposited onto each specimen with the air plasma spray (APS) technique. The presence of yttria leads to the formation of a "non-transformable" tetragonal phase, which avoids the phase transformation between tetragonal and monoclinic phase typical of pure zirconia; such transformation is undesirable because it is accompanied by a volume change, which produces stresses in the coating and potential detachment from the bond coat. Different compositions, with a greater percentage of stabilizer, can be used, as well as several other compositions, normally applied as a second ceramic insulating layer on top of the usual one.

The thermal insulating ceramic layer used in the specimens has a thickness equal to 0.5 mm and a porosity equal to 16%.

The thickness values reported above were obtained in the metallographic section at a temperature of 20 °C by an optical microscope with a graduated scale in the eyepiece.

The specimens described above underwent cyclic oxidation tests in a furnace and (simulated) brazing heat treatment tests.

The cyclic oxidation tests were carried out according to a procedure whose characteristics are reported below:
- A tubular furnace was used, operated manually for the introduction and removal of the specimens, set to 1100 °C.
- Daily cycles were performed, leaving the specimens in the furnace for 23 hours and out of the furnace for 1 hour each day, with visual inspection. In this way, 4 cycles per week were performed.
- Over the weekend and Monday, the specimens remained in the furnace for 71 hours and on Monday out of the furnace for 1 hour.
- Each week, the specimens remained at a high temperature for 163 hours and underwent 5 cooling cycles to room temperature.
- The test ended with the detachment of the thermal insulating ceramic layer. The exposure time at high temperature that caused such detachment constituted the result, referred to as "FCT life" (these tests are normally denoted by the acronym FCT, namely Furnace Cyclic Test).

The simulated brazing test was performed by placing the specimens in an industrial furnace together with a filler of actual components undergoing brazing treatment (typically between 1150 and 1190 °C). The specimens were not in contact with the brazing alloy, but were at the same temperature and in the same atmosphere as the actual components, thus undergoing the same contamination risk.

### TEST RESULTS

Table II reports the results of the FCT test on the 6 specimens in Table I. For a proper evaluation of the results in Table II, the related deposition technique used must be taken into account. In fact, the low pressure plasma spray (LPPS) technique is more efficient but also more expensive and available from only a few suppliers, as well as less suitable for coating components that already have cooling holes (for example, used and repaired components that need to be re-coated before a second operational life); while the HVOF + APS flash technique is less expensive and readily available from all coating manufacturers for gas-turbine components.

**Table II**

| Specimen | FCT life (h) | | | Average |
|---|---|---|---|---|
| 1 | 3588 | 4008 | 4148 | 3915 |
| 2 | 3507 | 3565 | 3588 | 3553 |
| 3 | 3387 | 3527 | 3550 | 3488 |
| 4 | 3573 | 3876 | 3993 | 3814 |
| 5 | 3527 | 3667 | 3667 | 3620 |
| 6 | 3461 | 3461 | 3565 | 3496 |

For a more immediate display of the results, the values in Table II are also reported in the chart in Figure 2.

### COMMENTARY ON THE RESULTS

With regard to the bond coats deposited with the more expensive LPPS technique, the specimens 1 and 2 of the present invention, whose results are represented by the first two columns of the chart in Figure 2, are improved in terms of cyclic oxidation resistance (FCT test) compared to the reference with uniform composition (column 6).

With regard to the bond coats deposited with the HVOF + APS flash technique (columns 3, 4, and 5 of the chart in Figure 2), which is less expensive, more readily available, and more suitable for repairing and restoring components that have already been used, it can be seen that the results obtained were either comparable or higher to reference 6. In this regard, it should be considered that the HVOF + APS flash technique produces surface layers that are already partially oxidized, and thus perform inherently less with the same powder composition than those produced with LPPS.

The simulated brazing test compared the bond coat 6 (Amperit 418.117/Amperit 418.715, all LPPS) with bond coat 1 (Amperit 418.117/Amperit 436, all LPPS) and showed that, by using an aluminum-rich composition for the second layer, the formation of a reaction layer mainly made up of chromium carbide, which is brittle and poorly adapted to maintain the adhesion of the overlying ceramic insulating layer, is avoided.

In the case of comparison bond coat 6, an uneven layer of Cr23C6 particles was visible, and immediately below it, a blackish aluminum oxide layer mixed with other oxides. Further below, a thicker area being lower in chromium is visible, as such element is spread onto the surface to form the unwanted reaction layer.

In contrast, in the case of the bond coat 1 of the invention, no microstructure formed by chromium carbide was visible under the optical microscope, while under the electron microscope a very thin layer (about 0.5 µm) of dense aluminum oxide was visible on the surface.

## Claims

1. A thermal barrier fixed to a surface of a material exposed to high temperatures; said thermal barrier comprising a bond coat layer fixed to the surface of the material to be protected and a thermal insulating ceramic layer fixed to the bond coat layer; said thermal barrier being **characterized in that** said bond coat comprises a first and a second layer distinct from each other and both composed of a MCrAlY+N alloy; wherein M is selected from Ni and Co, and N is selected from the group composed of Re, Ir, Si, Ta and Pt;
- said first and second layers having a different % by weight of the elements;
- said first layer being in contact with said surface of the material to be protected and composed of 2 to 7% by weight of Al, 0.5 to 2% by weight of Y, 10 to 35% by weight of Cr, 0 to 5% by weight of N and a % by weight of M to complete 100;
- said second layer being fixed to said first layer and composed of 8 to 14% by weight of Al, 0.5 to 2% by weight of Y, 10 to 20% by weight of Cr, 0 to 5% by weight of N and a % by weight of M to complete 100;
- said first layer having a thickness between 100 and 500 µm and said second layer having a thickness less than or equal to 150 µm.

2. The thermal barrier according to claim 1, **characterized in that** said first layer has a thickness between 180 and 300 µm.

3. The thermal barrier according to claim 1 or 2, **characterized in that** said second layer has a thickness between 10 and 70 µm.

4. The thermal barrier according to one of the preceding claims, **characterized in that** said second layer has a surface with a roughness Ra between 8 and 23 µm.

5. The thermal barrier according to one of the preceding claims, **characterized in that** said second layer has a surface with a roughness Ra between 12 and 20 µm.

6. The thermal barrier according to one of the preceding claims, **characterized in that** said first layer is composed of 4 to 6% by weight of Al, 0.5 to 1% by weight of Y, 20 to 28% by weight of Cr, 0 to 2.5% by weight of N and a % by weight of M to complete 100.

7. The thermal barrier according to one of the preceding claims, **characterized in that** said second layer is composed of 10 to 12% by weight of Al, 0.5 to 1% by weight of Y, 13 to 17% by weight of Cr, 0 to 2.5% by weight of N and a % by weight of M to complete 100.
